

## UNITED STATES PATENT OFFICE

2,534,326

## PROCESS OF MANUFACTURING PHOTOGRAPHIC ELEMENTS

Clay Weaver, Wilmington, Del., assignor to E. I. du Pont de Nemours & Company, Wilmington, Del., a corporation of Delaware

No Drawing. Application November 27, 1946,  
Serial No. 712,721

5 Claims. (Cl. 117—34)

1

This invention relates to photographic elements bearing gelled layers of synthetic hydroxyl polymer-silver halide emulsions and to processes of preparing the same.

The coating of synthetic hydroxyl polymer-silver halide emulsions in thin, uniform layers is quite difficult to carry out on a continuous commercial scale. Such emulsions do not gel or set like gelatin with slight variations in temperature. When heat is used to drive off the solvent, the layers can be coated fairly rapidly but are not uniform in thickness. It has been proposed to add various types of gelling agents to polyvinyl alcohol compositions to improve their coating properties. They are generally added during the preparation of the emulsion. This practice, while useful for small-scale operations, has some disadvantages for large-scale commercial operations. The emulsions often gel or set up in the containers or coating apparatus and continued contact with the agents causes a change in photographic properties. The layers lack uniformity because the gelling agents continue to act upon storage.

An object of this invention is to provide improvements in the art of coating synthetic hydroxyl polymer layers and especially silver halide emulsions. A further object is to provide a simple process for controlling the gelling of silver halide hydroxyl polymer emulsion layers. A still further object is to provide such a process which can be used on a continuous commercial scale. Still other objects will be apparent from the following description of the invention.

It has been discovered, and this is the basis of the present invention, that gelled synthetic hydroxyl polymer layers and especially silver halide synthetic hydroxyl polymer silver salt emulsion layers having good surface characteristics and quality can be made by coating fluid mixtures of such polymers and silver halide emulsions having a pH greater than 7.0 onto a layer comprising substantial amounts of a soluble boron compound which forms a borate ion in aqueous solution, e. g., boric acid and its esters and salts. The boron compounds are preferably incorporated in a hydrophilic colloid layer which has good adherence to synthetic hydroxyl polymers. It is preferably composed of a synthetic hydroxyl polymer. The hydrophilic colloid layer containing the boron compound may be deposited directly on the support or on an anchoring substratum.

A silver halide emulsion or dispersion in various types of water-soluble to hydrophilic synthetic

2

hydroxyl polymers, for example, can be readily gelled by coating such an emulsion onto a layer containing a boron compound as specified above. The pH of the coated emulsion layer should be greater than 7. This can be accomplished by adjusting the pH of the sublayer and emulsion before coating. The soluble boron compound apparently diffuses into the silver halide emulsion layer and under the alkaline conditions there encountered causes the silver halide emulsion to gel or set at a rapid rate. The gelling takes effect progressively from the bottom upwards. After drying has been completed, it is smooth, hard, uniform, and of excellent quality. Emulsion coatings of the usual thickness are gelled or set in accordance with this invention in a matter of a few seconds.

By synthetic hydroxyl polymer is meant a linear polymer containing a plurality of recurring intralinear vinyl alcohol ( $-\text{CH}_2-\text{CHOH}-$ ) groups.

Synthetic hydroxyl polymers of the water-soluble to hydrophilic type including polyvinyl alcohol and its partially hydrolyzed water-soluble lower fatty acid esters, lower alkyl ethers, and lower acetals have been proposed as silver halide binding agents for photographic elements. Polyvinyl alcohol is a tough, water-white, polymeric film-forming material. It is soluble in water. The more highly polymerized varieties are soluble in hot water and the medium or lower polymers are soluble in cold water. They are usually prepared by hydrolysis of polyvinyl esters, such as polyvinyl acetate, polyvinyl chloracetate, polyvinyl isobutyrate, etc. The partly hydrolyzed esters which contain a large number of recurring vinyl alcohol units ( $-\text{CH}_2-\text{CHOH}-$ ) are water-soluble in character. The ethers can be made by incompletely etherifying the completely or partially hydrolyzed polyvinyl acetate, etc. The polyvinyl acetals, e. g., polyvinyl acetaldehyde acetal and polyvinyl isobutyral, can be made by acetalization of polyvinyl alcohol and its incompletely hydrolyzed carboxylic acid esters.

In addition to the water-soluble and hydrophilic synthetic hydroxyl polymers just described, there may be mentioned partially and completely hydrolyzed polyvinyl esters, e. g., vinyl acetate and copolymers thereof with ethylenically unsaturated compounds, such as vinyl chloride and styrene; acrylic acid esters, e. g., methyl acrylate; methacrylic acid esters, e. g., methyl methacrylate; and mono-olefines, e. g., ethylene. The completely hydrolyzed ethylene/vinyl acetate copolymer emulsion described in McQueen 2,397,866 and Roland 2,386,347 form an important class

of silver halide emulsions which can advantageously be coated by the improved methods in question. These polymers may contain color-former nuclei. Suitable polymers of this latter type are described in United States Patents 2,310,943 and 2,320,422 and in United States applications Serial Numbers 528,946 now Patent Number 2,415,381 and 528,943 now Patent Number 2,397,865.

When a synthetic hydroxyl polymer is used as the colloid for the sublayer it is necessary to adjust the pH of the coating solution to 7.0 or lower so that uniform sublayers can be formed. This may be accomplished by the addition of small amounts of a readily soluble acid, e. g., glycolic acid, acetic acid, diglycolic acid, etc., or acid reacting salts, e. g., ammonium nitrate and ammonium chloride.

The soluble boron compounds are used in amounts sufficient to give complete gelling of the over-coated synthetic hydroxyl polymer-silver halide emulsion layer. The amounts, of course, vary in accordance with the particular hydroxyl polymer emulsion to be gelled. In general, amounts from 20 to 60% by weight of the polymer to be coated onto the sublayer are sufficient to gel the silver halide emulsion coatings.

The soluble boron compounds may be deposited directly on the support, e. g., paper, metal, synthetic resin, or super polymer, cellulose derivative, glass, etc., from an aqueous solution or dispersion or from a solvent or onto a sublayer which has good anchorage characteristics.

The invention will be further illustrated but is not intended to be limited by the following examples. The parts are by weight.

#### Example I

A hydrolyzed ethylene/vinyl acetate interpolymer of the type described in Example I of United States Patent 2,397,866 in an amount of one part was dissolved in a mixture of 40 parts of ethanol and 60 parts of water. One-tenth part of boric acid and one-tenth part of diethylene glycol were added and the resulting mixture coated onto a cellulose acetate film base and the resulting layer was dried. A light-sensitive emulsion containing silver halide grains dispersed in the same type of hydrophilic interpolymer and having a pH of 8 to 9 was coated onto the sublayer. The emulsion gelled rapidly when applied and a smooth coating was obtained.

Similar results can be obtained by substituting for the boric acid equivalent amounts of boric acid esters, e. g., diethylene glycol borate, mannitol borate, etc.

#### Example II

A double weight raw paper is coated with a solution made by adding 7.58 grams of ammonium sulfate in 70.5 cc. of water to 470 grams of a 10% solution of the interpolymer set forth in Example I. To the mixture is added in thirty seconds 11.75 grams of barium chloride in 470 cc. of water, 3 cc. of an 0.5% solution of Monastral Blue BWD, 5 cc. of a 5% saponin solution, 200 cc. of a 10% aqueous solution of diethylene glycol borate, and 5.7 grams of glycolic acid. The coating is dried for 30 minutes at 40° C. One hundred cubic centimeters (100 cc.) of the silver halide emulsion described in Example I but containing 3 cc. of 6N KOH is coated onto the sublayer. Firm gelation of the emulsion layer occurs in 30 seconds.

The diethylene glycol borate of this ex-

ample can be made by reacting diethylene glycol, boric acid, and borax at 100° to 160° C. as described in United States Patent 1,953,741. It can also be replaced by an equivalent amount of boric acid and diethylene glycol.

#### Example III

Ten parts of an acetal of a hydrolyzed ethylene/vinyl acetate copolymer (ethylene/vinyl acetate ratio 1/10) with benzaldehyde-ortho-sulfonic acid prepared as described in Example I of application Serial Number 551,801, filed August 30, 1944, now abandoned, and the continuation-in-part thereof Serial Number 698,799, filed September 23, 1946, now Patent Number 2,462,151 is dissolved in a mixture of 25 parts of water and 175 parts of methanol. To this is added a solution of three parts of boric acid and three parts of diethylene glycol in a mixture of 25 parts of water and 75 parts of methanol. This solution is then diluted to 1000 parts with a 50/50 mixture of methanol and ethanol. Cellulose nitrate film base is coated with this solution and after drying it is coated with a silver halide emulsion in hydrolyzed ethylene/vinyl acetate prepared as described in Example I of United States Patent 2,397,866 and having a pH of 7.5. Within 30 seconds after coating this emulsion layer sets to a firm gel which can be dried rapidly to a smooth, uniform, light-sensitive layer.

#### Example IV

Ten parts of the mixed polyvinyl acetal of salicylaldehyde and phthalaldehydic acid, prepared as described in Example III of United States Patent 2,310,943, is used in place of the acetal of Example III hereof to form a substratum layer. Over this is coated a silver halide emulsion prepared in the polyvinyl acetal of salicylaldehyde as described in United States Patent 2,397,864, Example IV. The resulting light-sensitive coating is smooth and uniform and exhibits good anchorage, dry and wet.

#### Example V

A subbed film base, prepared as in Example III, is coated with a 4% solution of hydrolyzed ethylene/vinyl acetate (see Example I of United States Patent 2,397,866) in ethanol/water (20/80) containing 4% by weight of comminuted silver. This non-halation layer dries to a smooth, uniform, light-absorbing film. In place of the comminuted silver, non-halation dyes may be used. Suitable dyes are described in United States Patent 2,203,767.

In place of the specific gelling agents described above, there may be substituted other boric acid esters or salts capable of yielding borate ions in aqueous solution. Suitable additional compounds include sodium and potassium tetraborate, metaborate, and orthoborate, boric acid, glyceryl borate, glycerol boroborate; the sorbitol, mannitol, and dulcitol monoborate and diborates and mono- and poly-condensation products and their sodium and ammonium salts set forth in Examples 1 to 19 of United States Patent 2,223,349 and Examples 3, 4, 5, 7, 9, 14, and 18 to 35 of United States Patent 2,223,948. Moreover, suitable boric acid esters can be prepared by reacting a polyhydric alcohol, e.g., ethylene glycol, diethylene glycol, triethylene glycol, erythrol, sorbitol, and mannitol with boric acid or a mixture of boric acid and borax, by heating the admixture to 100° to 160° C. A copious

evolution of water occurs. The resulting products are viscous syrups or resins of a colloidal nature and have a high molecular weight and complex structure. They are readily soluble in water but are substantially insoluble in hydrocarbons. Their preparation is described in various United States Patents including 1,953,741, 2,223,349, 2,223,948, 2,223,949, and 2,224,011. These compounds have been referred to as boraborates.

The invention is not limited to the use of the gelling agents in a colloid substratum layer. Aqueous solutions of the gelling agents may be deposited directly on a support and the layer or coating to be gelled deposited thereon. In the case of hydrophobic supports, the anchorage is not sufficient for permanency. However, good strippable gelled emulsion layers can be made by the latter technique. The gelling sublayers can be used to gel other types of overcoatings than the silver halide emulsion layers described above. Thus clear colloid layers, filter layers, and anti-halation layers utilizing synthetic hydroxyl polymer binding agents can be coated in like manner. In the case of photographic papers, the sublayer containing the boron compound may also contain a pigment, e.g., baryta. In such cases alkaline agents may be added to the coating solutions to adjust the pH to more than 7.

Various water-miscible materials, such as solvents and/or crystallization inhibitors, may be added to the coating solutions for the gelling sublayers. Suitable such materials include ethanol, methanol, isopropanol, tertiary butanol, dioxane, ethylene glycol, diethylene glycol, mannitol, the monomethyl ether of ethylene glycol, dimethylformamide, formamide, acetone, and dioxolane.

Various types of hydrophilic colloids may be used as binding media for the gelling agents including not only the synthetic hydrophilic hydroxyl polymers and colloids above-described but also galatin, casein, methyl cellulose, and the hydrophilic polyvinyl acetals containing solubilizing groups described in Woodward application Serial Number 551,801, filed August 30, 1944, now abandoned, and the continuation-in-part thereof Serial Number 698,799, filed September 23, 1946 now Patent Number 2,462,151.

The invention is useful in the preparation of photographic elements for various purposes. Thus it is useful in the preparation of photographic elements, such as motion picture and portrait films, lithographic film, printing plates, photographic papers, etc.

The invention is especially advantageous with supports which are difficult to coat. It can be used on cellulose nitrate, cellulose acetate, cellulose propionate, cellulose acetate-propionate, cellulose acetate butyrate, polyvinyl chloride, glass, metal, regenerated cellulose, super polyamides (nylon), polyvinyl fluorides, etc.

An advantage of the invention is that it provides a simple method for gelling synthetic hydroxyl polymer silver halide emulsion layers. A further advantage is that the gelling of such layers can be efficiently controlled. A still further advantage is that it simplifies coating operations in that the emulsions do not substantially vary in viscosity during coating operations. Since the gelling agents are not added to the coating solutions of the silver halide emulsions, there is no danger of having them set up or gel prior to coating. A further advantage resides in the fact that no color is imparted from

the novel gelling agents. The gelling takes effect from the bottom of the coated layer upwardly giving a uniform product. The action is very rapid and gelling takes place as the coating solution is applied to the layer containing the gelling agent. Another advantage is the avoidance of undesirable photographic changes in the applied emulsion.

As many apparently widely different embodiments of this invention may be made without departing from the spirit and scope thereof, it is to be understood that the invention is not to be limited except as defined by the appended claims.

15. What is claimed is:

1. A process of manufacturing photographic elements which comprises coating a support with a solution of a synthetic hydroxyl polymer containing a substantial amount of a soluble boron compound capable of yielding borate ions, said solution having a pH less than 7.0, drying the layer and coating the resulting layer with a fluid silver halide emulsion in a synthetic hydroxyl polymer having a pH greater than 7.0, each said hydroxyl polymer being water-soluble to hydrophilic in character and containing a large number of recurring intralinear



30 groups.

2. A process of manufacturing photographic elements which comprises coating a support with a solution of a synthetic hydroxyl polymer containing a substantial amount of boric acid, said solution having a pH less than 7.0, drying the layer and coating the resulting layer with a fluid silver halide emulsion in a synthetic hydroxyl polymer having a pH greater than 7.0, each said hydroxyl polymer being water-soluble to hydrophilic in character and containing a large number of recurring intralinear



groups.

3. A process of manufacturing photographic film elements which comprises coating a film base with a solution of a synthetic hydroxyl polymer containing a substantial amount of a soluble boron compound capable of yielding borate ions, said solution having a pH less than 7.0, drying the layer and coating the resulting layer with a fluid silver halide emulsion in a synthetic hydroxyl polymer having a pH greater than 7.0, each said hydroxyl polymer being water-soluble to hydrophilic in character and containing a large number of recurring intralinear



groups.

4. A process of manufacturing photographic film elements which comprises coating a film base with a solution of polyvinyl alcohol containing a substantial amount of a soluble boron compound capable of yielding borate ions, said solution having a pH less than 7.0, drying the layer and coating the resulting layer with a fluid silver halide emulsion in polyvinyl alcohol having a pH greater than 7.0.

5. A process of manufacturing photographic elements which comprises coating a paper support with a solution of a hydrophilic hydrolyzed ethylene/vinyl acetate copolymer containing finely divided baryta and a soluble boron compound capable of yielding borate ions, said solution having a pH less than 7.0, drying the layer and coating the resulting layer with a fluid silver

halide emulsion in a hydrophilic hydrolyzed ethylene/vinyl acetate copolymer having a pH greater than 7.0 each of said copolymers containing a large number of recurring intralinear

groups.



CLAY WEAVER.

## UNITED STATES PATENTS

|   | Number    | Name        | Date          |
|---|-----------|-------------|---------------|
|   | 2,249,538 | McDowell    | July 15, 1941 |
|   | 2,251,296 | Shipp       | Aug. 5, 1941  |
| 5 | 2,376,371 | Lowe et al. | May 22, 1945  |
|   | 2,386,347 | Roland      | Oct. 9, 1945  |
|   | 2,397,866 | McQueen     | Apr. 2, 1946  |

## REFERENCES CITED

The following references are of record in the file of this patent: